

M. B. BECKER.

METHOD OF ORNAMENTING PREPARED ROOFING.

APPLICATION FILED FEB. 1, 1912.

1,024,549.

Patented Apr. 30, 1912.

2 SHEETS-SHEET 1.



Witnesses:

G. W. Marus Jr.

R. Burkhardt.

Intendant

Mathias B. Becker  
By: Rudolph J. J. Betty

M. B. BECKER.

METHOD OF ORNAMENTING PREPARED ROOFING.

APPLICATION FILED FEB. 1, 1912.

1,024,549.

Patented Apr. 30, 1912.

2 SHEETS-SHEET 2.

FIG. 2.



FIG. 3.



Witnesses:

G. W. Buarus Jr.

P. Burkhardt.

Inventor

Mathias B. Becker

By: Rudolph J. D. B.

Atty

# UNITED STATES PATENT OFFICE.

MATHIAS B. BECKER, OF CHICAGO, ILLINOIS.

## METHOD OF ORNAMENTING PREPARED ROOFING.

1,024,549.

Specification of Letters Patent.

Patented Apr. 30, 1912.

Application filed February 1, 1912. Serial No. 674,820.

*To all whom it may concern:*

Be it known that I, MATHIAS B. BECKER, citizen of the United States, residing at Chicago, in the county of Cook and State 5 of Illinois, have invented certain new and useful Improvements in Methods of Ornamenting Prepared Roofing; and I do hereby declare the following to be a full, clear, and exact description of the invention, such 10 as will enable others skilled in the art to which it appertains to make and use the same.

This invention has for its object to provide a novel method of producing prepared 15 roofing and consists in the steps hereinafter fully described and claimed.

In the accompanying drawings: Figure 1— is a view in central vertical longitudinal section of a machine employed in 20 carrying out my said process. Fig. —2— is a fragmentary view in elevation of roofing prepared in accordance with my process. Fig. —3— is a detail sectional view of the roofing on the line 3—3 of Fig. —2—.

25 The object of my present invention is to provide a process for treating prepared roofing whereby a design in different colors is produced thereon while at the same time the life and wearing qualities of the roofing are materially increased. The product resulting from carrying out this process is 30 fully described and claimed in a companion application filed of even date herewith, Serial No. 674,821.

35 Prepared roofing usually consists of a sheet or web A of wool felt or other fibrous material which is impregnated with and provided with surface coatings B and C of asphaltum. Upon the coating B there is 40 applied a covering of granulated grit particles D such as gravel, crushed stone or slate which is applied while said coating is hot and soft and becomes partially embedded therein. The character or color of 45 such grit determines the color of the roof to which the material is applied, such color being uniform and rather monotonous in appearance.

50 My said process consists in applying upon certain predetermined fields of the grit coated surface of the roofing a liquid having the quality of being water-proof when dry and capable of adhering to the asphaltum

coating in which the grit is partially embedded and in such quantity as to substantially embed said grit coating and become amalgamated or homogeneous with the asphaltum coating underneath the same so as to so completely and thoroughly attach such grit to said asphaltum coating as 60 to prevent the same from being washed away by rain or carried away by snow and ice.

In carrying out my process I prefer to employ a dilute asphaltum, that is asphaltum admixed while hot with creosote or benzin, this being effected by heating the asphaltum to a temperature of 450 degrees Fahr. more or less, and pouring the same, while at this temperature, into 70 a tank containing benzin or creosote, the latter becoming thoroughly admixed and intermingled with said asphaltum immediately upon contact of the two, it being obvious, of course, that a relatively large 75 proportion of said benzin or creosote will pass off in vapor while the process of commingling is going on. The resulting liquid consists substantially of seventy (70) per cent., more or less, asphaltum and thirty 80 (30) per cent., more or less, creosote or benzin, depending upon which of these two substances is used.

Benzin and creosote are known solvents of asphaltum and the resulting mixtures when 85 applied either hot or cold to the asphaltum surface of the prepared roofing will cause the latter to partially dissolve and when dry the coating E applied in liquid form will become substantially homogeneous and 90 firmly amalgamated with the asphaltum coating of the prepared roofing.

The fluent asphaltum may be applied upon the grit coated surface of the prepared roofing in any desired manner, as for example, 95 by means of stencils or by means of an ordinary paint brush either with or without the use of a stencil. However, this method of applying the same is necessarily very expensive and would so increase the 100 cost of the roofing as to render it prohibitive in competition with the more expensive and more attractive kinds of roofing.

In order to cheaply produce the design on the roofing in such a manner as to cause 105 the amalgamation before referred to to be

effected, I prefer to employ a machine for the purpose which is fully described in a companion application filed of even date herewith Serial No. 674,819. The said machine is equipped with a rotating cylinder 1 having its surface divided into fields of such shape as it may be desired to reproduce on the roofing, as for example, the diamond shape fields shown in the drawings. On 10 each field of the circumferential face of the cylinder 1 there is mounted a pad 2 of a spongy absorbent material, such for example, as thick wool felt, the pads of the latter being adapted to be brought into surface 15 contact with the grit coated face of the roofing by compressing the latter against the cylinder during rotation of the latter and travel of the former, this being effected by means of a second cylinder 3 bearing on the 20 other face of the roofing and serving to compress the same against said pads 2. Below the cylinder 1 there is mounted a pan 4 containing the dilute asphaltum in which the pads 2 carried by the cylinder become immersed during the revolution of the cylinder and of which they absorb a relatively 25 large quantity. As said pads 2 are compressed against the grit coated surface of the roofing, the grit particles embed themselves in the surfaces of said pads and by 30 the compression of the latter the liquid is expelled as from a sponge and thus a sufficient quantity applied to the grit coated surface to completely coat each grit particle and 35 penetrate through the grit coating into contact with the asphaltum coating with which it amalgamates and becomes homogeneous.

The dilute asphaltum is preferably applied cold to the cool roofing but if found 40 desirable either or both may be heated without departing from the invention.

The dilute asphaltum is black and will produce black fields on grit coating. Any other color of liquid having substantially 45 the same properties may be substituted for the dilute asphaltum without departing from the invention.

I claim as my invention:

1. The herein-described method of ornamenting prepared asphaltum roofing having 50 a grit coated surface, which consists in applying on various parts of the grit coated surface a solution of a substance having the property of dissolving the asphaltum coating and in drying to become amalgamated 55 therewith, said solution being waterproof when dry and being of a different color from the grit and applied in such quantity as to cover and penetrate through said grit coating and envelop the grit particles. 60

2. The herein-described method of ornamenting prepared asphaltum roofing having a grit coated surface, which consists in applying on various parts of the grit coated surface a cool solution of a substance having 65 the property of dissolving the asphaltum coating and in drying to become amalgamated therewith, said solution being waterproof when dry and being of a different color from the grit and applied in such 70 quantity as to cover and penetrate through said grit coating and envelop the grit particles.

3. The herein-described method of ornamenting prepared asphaltum roofing having 75 a grit coated surface, which consists in applying on various parts of the grit coated surface of the roofing when cool, a cool solution of a substance having the property of dissolving the asphaltum coating and in 80 drying to become amalgamated therewith, said solution being waterproof when dry and being of a different color from the grit and applied in such quantity as to cover and penetrate through said grit coating and 85 envelop the grit particles.

In testimony whereof I have signed my name in presence of two subscribing witnesses.

MATHIAS B. BECKER.

Witnesses:

M. M. BOYLE,  
RUDOLPH WM. LOTZ.